



US008062816B2

(12) **United States Patent**  
**Wu**

(10) **Patent No.:** **US 8,062,816 B2**  
(45) **Date of Patent:** **Nov. 22, 2011**

(54) **PHOSPHONATE HOLE BLOCKING LAYER  
PHOTOCODUCTORS**

(75) Inventor: **Jin Wu**, Webster, NY (US)

(73) Assignee: **Xerox Corporation**, Norwalk, CT (US)

(\*) Notice: Subject to any disclaimer, the term of this patent is extended or adjusted under 35 U.S.C. 154(b) by 827 days.

(21) Appl. No.: **12/129,977**

(22) Filed: **May 30, 2008**

(65) **Prior Publication Data**

US 2009/0297967 A1 Dec. 3, 2009

(51) **Int. Cl.**  
**G03G 5/00** (2006.01)

(52) **U.S. Cl.** ..... **430/58.8**; 430/60; 430/64

(58) **Field of Classification Search** ..... 430/64,  
430/58.05, 97, 57.1, 58.8

See application file for complete search history.

(56) **References Cited**

U.S. PATENT DOCUMENTS

|                   |         |                     |
|-------------------|---------|---------------------|
| 4,265,990 A       | 5/1981  | Stolka et al.       |
| 4,464,450 A       | 8/1984  | Teuscher            |
| 4,921,769 A       | 5/1990  | Yuh et al.          |
| 5,114,818 A *     | 5/1992  | Yu .....            |
| 5,385,796 A       | 1/1995  | Spiewak et al.      |
| 5,449,573 A       | 9/1995  | Aoki et al.         |
| 5,906,904 A       | 5/1999  | Parikh et al.       |
| 5,928,824 A       | 7/1999  | Obinata et al.      |
| 6,015,645 A       | 1/2000  | Murti et al.        |
| 6,156,468 A       | 12/2000 | Wehelie et al.      |
| 6,177,219 B1      | 1/2001  | Yuh et al.          |
| 6,255,027 B1      | 7/2001  | Wehelie et al.      |
| 6,913,863 B2      | 7/2005  | Wu et al.           |
| 7,312,007 B2      | 12/2007 | Lin et al.          |
| 2004/0115547 A1   | 6/2004  | Tong et al.         |
| 2005/0058919 A1 * | 3/2005  | Tong et al. .....   |
| 2005/0136349 A1 * | 6/2005  | Mishra et al. ..... |
| 2007/0026328 A1   | 2/2007  | Wu et al.           |
| 2007/0026330 A1 * | 2/2007  | Wu et al. .....     |
| 2007/0049677 A1   | 3/2007  | Wu et al.           |
| 2007/0243476 A1   | 10/2007 | Lin et al.          |
| 2008/0008947 A1   | 1/2008  | Wu                  |
| 2008/0032219 A1   | 2/2008  | Lin et al.          |
| 2009/0325091 A1 * | 12/2009 | Wu et al. .....     |

OTHER PUBLICATIONS

Jin Wu, U.S. Appl. No. 12/129,958 on Anthracene Containing Photoconductors, filed concurrently herewith.

Jin Wu, U.S. Appl. No. 12/129,965 on Ferrocene Containing Photoconductors, filed concurrently herewith.

Jin Wu, U.S. Appl. No. 12/129,969 on Amine Phosphate Containing Photogenerating Layer Photoconductors, filed concurrently herewith.

Jin Wu, U.S. Appl. No. 12/129,943 on Phenol Polysulfide Containing Photogenerating Layer Photoconductors, filed concurrently herewith.

Jin Wu, U.S. Appl. No. 12/129,948 on Aminosilane and a Self Crosslinking Acrylic Resin Hole Blocking Layer Photoconductors, filed concurrently herewith.

Jin Wu, U.S. Appl. No. 12/129,982 on Zirconocene Containing Photoconductors, filed concurrently herewith.

Jin Wu et al., U.S. Appl. No. 12/129,952 on Backing Layer Containing Photoconductor, filed concurrently herewith.

Jin Wu, U.S. Appl. No. 12/129,989 on Polymer Anticurl Backside Coating (ACBC) Photoconductors, filed concurrently herewith.

Jin Wu, U.S. Appl. No. 12/129,995 on Polyimide Intermediate Transfer Components, filed concurrently herewith.

Jin Wu, U.S. Appl. No. 12/059,536 on Carbazole Hole Blocking Layer Photoconductors, filed Mar. 31, 2008.

Jin Wu, U.S. Appl. No. 11/831,440 on Iron Containing Hole Blocking Layer Containing Photoconductors, filed Jul. 31, 2007.

Jin Wu, U.S. Appl. No. 11/831,453 on UV Absorbing Hole Blocking Layer Containing Photoconductors, filed Jul. 31, 2007.

Jin Wu, U.S. Appl. No. 11/831,476 on Indonium Hole Blocking Layer Photoconductors, filed Jul. 31, 2007.

Jin Wu, U.S. Appl. No. 11/831,469 on Copper Containing Hole blocking Layer Photoconductors, filed Jul. 31, 2007.

Jin Wu et al., U.S. Appl. No. 11/764,489 on Hole Blocking Layer Containing Photoconductors, filed Jun. 18, 2007.

Jin Wu et al., U.S. Appl. No. 11/714,600 on Hole Blocking Layer Containing Photoconductors, filed Mar. 6, 2007.

\* cited by examiner

*Primary Examiner* — Mark F Huff

*Assistant Examiner* — Rashid Alam

(74) *Attorney, Agent, or Firm* — Oliff & Berridge, PLC

(57) **ABSTRACT**

A photoconductor that includes, for example, a substrate; a first layer like a ground plane layer; an undercoat layer thereover wherein the undercoat layer contains an aminosilane and a phosphonate; a photogenerating layer; and at least one charge transport layer.

**30 Claims, No Drawings**

**PHOSPHONATE HOLE BLOCKING LAYER  
PHOTOCODUCTORS**

**CROSS REFERENCE TO RELATED  
APPLICATIONS**

U.S. application Ser. No. 12/129,958, U.S. Publication No. 20090297964 on Anthracene Containing Photoconductors, filed May 30, 2008, the disclosure of which is totally incorporated herein by reference.

U.S. application Ser. No. 12/129,965, U.S. Publication No. 20090297965 on Ferrocene Containing Photoconductors, filed May 30, 2008, the disclosure of which is totally incorporated herein by reference.

U.S. Application No. 12/129,969, U.S. Publication No. 20090297966 on Amine Phosphate Containing Photogenerating Layer Photoconductors, filed May 30, 2008, the disclosure of which is totally incorporated herein by reference.

U.S. application Ser. No. 12/129,943, U.S. Publication No. 20090297961 on Phenol Polysulfide Containing Photogenerating Layer Photoconductors, filed May 30, 2008, the disclosure of which is totally incorporated herein by reference.

U.S. application Ser. No. 12/129,948, U.S. Publication No. 20090297962 on Aminosilane and a Self Crosslinking Acrylic Resin Hole Blocking Layer Photoconductors, filed May 30, 2008, the disclosure of which is totally incorporated herein by reference.

U.S. application Ser. No. 12/129,982, U.S. Publication No. 20090297968 on Zirconocene Containing Photoconductors, filed May 30, 2008, the disclosure of which is totally incorporated herein by reference.

U.S. Application No. 12/129,952, U.S. Publication No. 20090297963 on Backing Layer Containing Photoconductor, filed May 30, 2008, the disclosure of which is totally incorporated herein by reference.

U.S. application Ser. No. 12/129,989, U.S. Publication No. 20090297969 on Polymer Anticurl Backside Coating (ACBC) Photoconductors, filed May 30, 2008, the disclosure of which is totally incorporated herein by reference.

U.S. application Ser. No. 12/129,995, U.S. Publication No. 20090297232 on Polyimide Intermediate Transfer Components, filed May 30, 2008, the disclosure of which is totally incorporated herein by reference.

Illustrated in U.S. application Ser. No. 12/059,536, now U.S. Pat. No. 7,794,906, filed Mar. 31, 2008, entitled Carbazole Hole Blocking Layer Photoconductors, the disclosure of which is totally incorporated herein by reference, is

Illustrated in U.S. application Ser. No. 11/831,440, now U.S. Pat. No. 7,871,748, filed Jul. 31, 2007, entitled Iron Containing Hole Blocking Layer Containing Photoconductors, the disclosure of which is totally incorporated herein by reference, is a photoconductor comprising a substrate; an undercoat layer thereover wherein the undercoat layer comprises a metal oxide, and an iron containing compound; a photogenerating layer; and at least one charge transport layer.

Illustrated in U.S. application Ser. No. 11/831,453, now U.S. Pat. No. 7,670,737, filed Jul. 31, 2007, entitled UV Absorbing Hole Blocking Layer Containing Photoconductors, the disclosure of which is totally incorporated herein by reference, is a photoconductor comprising a substrate; an undercoat layer thereover wherein the undercoat layer comprises a metal oxide, and an ultraviolet light absorber component; a photogenerating layer; and at least one charge transport layer.

Illustrated in U.S. application Ser. No. 11/831,476, now U.S. Pat. No. 7,851,115, filed Jul. 31, 2007, entitled Iodonium Hole Blocking Layer Photoconductor, the disclosure of

which is totally incorporated herein by reference, is a photoconductor comprising a substrate; an undercoat layer thereover wherein the undercoat layer comprises a metal oxide and an iodonium containing compound; a photogenerating layer; and at least one charge transport layer.

Illustrated in U.S. application Ser. No. 11/831,469, now U.S. Pat. No. 7,867,676, filed Jul. 11, 2007, entitled Copper Containing Hole Blocking Layer Photoconductors, the disclosure of which is totally incorporated herein by reference, is a photoconductor comprising a substrate; an undercoat layer thereover wherein the undercoat layer comprises a metal oxide, and a copper containing compound; a photogenerating layer; and at least one charge transport layer.

Illustrated in U.S. application Ser. No. 11/211,757, U.S. Publication No. 20070049677, now U.S. Pat. No. 7,544,452, filed Aug. 26, 2005, entitled Thick Electrophotographic Imaging Member Undercoat Layers, the disclosure of which is totally incorporated herein by reference, are binders containing metal oxide nanoparticles and a co-resin of phenolic resin and aminoplast resin, and an electrophotographic imaging member undercoat layer containing the binders.

Disclosed in U.S. application Ser. No. 11/764,489, now U.S. Pat. No. 7,846,628, filed Jun. 18, 2007, entitled Hole Blocking Layer Containing Photoconductors, the disclosure of which is totally incorporated herein by reference, is a photoconductor comprising a substrate; an undercoat layer thereover wherein the undercoat layer comprises a metal oxide, an electron donor, and an electron acceptor charge transfer complex; a photogenerating layer; and at least one charge transport layer.

Disclosed in U.S. application Ser. No. 11/403,981, U.S. Publication 20070243476, now U.S. Pat. No. 7,604,914, filed Apr. 13, 2006, entitled Imaging Members, the disclosure of which is totally incorporated herein by reference, is an electrophotographic imaging member, comprising a substrate, an undercoat layer disposed on the substrate, wherein the undercoat layer comprises a polyol resin, an aminoplast resin, and a metal oxide dispersed therein; and at least one imaging layer formed on the undercoat layer, and wherein the polyol resin is, for example, selected from the group consisting of acrylic polyols, polyglycols, polyglycerols, and mixtures thereof.

Illustrated in U.S. patent application Ser. No. 11/481,642, U.S. Publication 20080008947, now U.S. Pat. No. 7,732,112, filed Jul. 6, 2006, the disclosure of which is totally incorporated by reference herein, is an imaging member including a substrate; a charge generation layer positioned on the substrate; at least one charge transport layer positioned on the charge generation layer; and an undercoat or hole blocking layer positioned on the substrate on a side opposite the charge generation layer, the undercoat layer comprising a binder component and a metallic component comprising a metal thiocyanate and metal oxide.

Disclosed in U.S. Application No. 11/496,790, U.S. Publication 20080032219, now U.S. Pat. No. 7,560,208, filed Aug. 1, 2006, the disclosure of which is totally incorporated herein by reference, is a photoconductor member comprising a substrate; an undercoat layer thereover wherein the undercoat layer comprises a polyol resin, an aminoplast resin, a polyester adhesion component and a metal oxide; and at least one imaging layer formed on the undercoat layer.

Disclosed in U.S. application Ser. No. 11/714,600, now U.S. Pat. No. 7,579,126, filed Mar. 6, 2007, the disclosure of which is totally incorporated herein by reference, is a photoconductor comprising a substrate; an undercoat layer thereover wherein the undercoat layer comprises an electrocon-

ducting component dispersed in a rapid curing polymer matrix; a photogenerating layer, and at least one charge transport layer.

The appropriate components and processes, number and sequence of the layers, component and component amounts in each layer, and the thicknesses of each layer of the above copending applications, may be selected for the present disclosure photoconductors in embodiments thereof.

## BACKGROUND

There are disclosed herein hole blocking layers, and more specifically, photoconductors containing a hole blocking layer or undercoat layer (UCL) comprised, for example, of an aminosilane and a phosphonate, and which layer is coated or deposited on a first layer like a ground plane layer of, for example, gold or a gold containing compound.

In embodiments, photoconductors comprised of the disclosed hole blocking or undercoat layer enables, for example, the blocking of or minimization of the movement of holes or positive charges generated from the ground plane layer; excellent cyclic stability, and thus color print stability especially for xerographic generated color copies. Excellent cyclic stability of the photoconductor refers, for example, to almost no or minimal change in a generated known photoinduced discharge curve (PIDC), especially no or minimal residual potential cycle up after a number of charge/discharge cycles of the photoconductor, for example about 200 kilocycles, or xerographic prints of, for example from about 80 to about 200 kiloprints. Excellent color print stability refers, for example, to substantially no or minimal change in solid area density, especially in 60 percent halftone prints, and no or minimal random color variability from print to print after a number of xerographic prints, for example 50 kiloprints.

Further, in embodiments the photoconductors disclosed may, it is believed, possess the minimization or substantial elimination of undesirable ghosting on developed images, such as xerographic images, including improved ghosting at various relative humidities; excellent cyclic and stable electrical properties; acceptable charge deficient spots (CDS); and compatibility with the photogenerating and charge transport resin binders, such as polycarbonates. Charge blocking layer and hole blocking layer are generally used interchangeably with the phrase "undercoat layer".

The need for excellent print quality in xerographic systems is of value, especially with the advent of color. Common print quality issues can be dependent on the components of the undercoat layer (UCL). In certain situations, a thicker undercoat is desirable, but the thickness of the material used for the undercoat layer may be limited by, in some instances, in view of the inefficient transport of the photoinjected electrons from the generator layer to the substrate. When the undercoat layer is too thin, then incomplete coverage of the substrate may sometimes result due to wetting problems on localized unclean substrate surface areas. This incomplete coverage may produce pin holes which can, in turn, produce print defects such as charge deficient spots (CDS) and bias charge roll (BCR) leakage breakdown. Other problems include image "ghosting" resulting from, it is believed, the accumulation of charge somewhere in the photoreceptor. Removing trapped electrons and holes residing in the imaging members is a factor in preventing ghosting. During the exposure and development stages of xerographic cycles, the trapped electrons are mainly at or near the interface between the charge generation layer (CGL) and the undercoat layer (UCL), and holes are present mainly at or near the interface between the charge generation layer and the charge transport layer (CTL).

The trapped charges can migrate according to the electric field during the transfer stage where the electrons can move from the interface of CGL/UCL to CTL/CGL, or the holes from CTL/CGL to CGL/UCL, and become deep traps that are no longer mobile. Consequently, when a sequential image is printed, the accumulated charge results in image density changes in the current printed image that reveals the previously printed image. Thus, there is a need to minimize or eliminate charge accumulation in photoreceptors without sacrificing the desired thickness of the undercoat layer, and a need for permitting the UCL to properly adhere to the other photoconductive layers, such as the photogenerating layer, for extended time periods, such as for example, about 1,000, 000 simulated xerographic imaging cycles. Thus, a number of conventional materials used for the undercoat or blocking layer possesses a number of disadvantages resulting in adverse print quality characteristics. For example, ghosting, charge deficient spots, and bias charge roll leakage breakdown are problems that commonly occur. With regard to ghosting, which is believed to result from the accumulation of charge somewhere in the photoconductor, consequently, when a sequential image is printed, the accumulated charge results in image density change in the current printed image that reveals the previously printed image.

Thick undercoat layers are sometimes desirable for xerographic photoconductors as such layers permit photoconductor life extension and carbon fiber resistance. Furthermore, thicker undercoat layers permit the use of economical substrates in the photoreceptors. Examples of thick undercoat layers are disclosed in U.S. Pat. No. 7,312,007, the entire disclosure of which is totally incorporated herein by reference. However, due primarily to insufficient electron conductivity in dry and cold environments, the residual potential in conditions, such as 10 percent relative humidity and 70° F., can be high when the undercoat layer is thicker than about 15 microns, and moreover, the adhesion of the UCL may be poor, disadvantages avoided or minimized with the UCL of the present disclosure.

Also included within the scope of the present disclosure are methods of imaging and printing with the photoconductive devices illustrated herein. These methods generally involve the formation of an electrostatic latent image on the imaging member, followed by developing the image with a toner composition comprised, for example, of a thermoplastic resin, colorant, such as pigment, charge additive, and surface additives, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same operation with the exception that exposure can be accomplished with a laser device or image bar. More specifically, the imaging members, photoconductor drums, and flexible belts disclosed herein can be selected for the Xerox Corporation iGEN3® machines that generate with some versions over 100 copies per minute. Processes of imaging, especially xerographic imaging and printing, including digital, and/or high speed color printing, are thus encompassed by the present disclosure.

The photoconductors disclosed herein are in embodiments sensitive in the wavelength region of, for example, from about 400 to about 900 nanometers, and in particular from about 650 to about 850 nanometers, thus diode lasers can be selected as the light source.

## REFERENCES

Illustrated in U.S. Pat. No. 7,312,007, the disclosure of which is totally incorporated herein by reference, is a photo-

conductive member containing a hole blocking layer, a photogenerating layer, and a charge transport layer, and wherein the hole blocking layer contains a metallic component like a titanium oxide and a polymeric binder.

Illustrated in U.S. Pat. No. 6,913,863, the disclosure of which is totally incorporated herein by reference, is a photoconductive imaging member comprised of an optional supporting substrate, a hole blocking layer thereover, a photogenerating layer, and a charge transport layer, and wherein the hole blocking layer is comprised of a metal oxide, a mixture of phenolic resins, and wherein at least one of the resins contains two hydroxy groups.

Illustrated in U.S. Pat. Nos. 6,255,027; 6,177,219, and 6,156,468, each of the disclosures thereof being totally incorporated herein by reference, are, for example, photoreceptors containing a charge blocking layer of a plurality of light scattering particles dispersed in a binder, reference for example, Example I of U.S. Pat. No. 6,156,468, wherein there is illustrated a charge blocking layer of titanium dioxide dispersed in a specific linear phenolic binder of VARCUM®, available from OxyChem Company.

Illustrated in U.S. Pat. No. 6,015,645, the disclosure of which is totally incorporated herein by reference, is a photoconductive imaging member comprised of a supporting substrate, a hole blocking layer, an optional adhesive layer, a photogenerating layer, and a charge transport layer, and wherein the blocking layer is comprised of a polyhaloalkylstyrene.

Layered photoconductors have been described in numerous U.S. patents, such as U.S. Pat. No. 4,265,990, the disclosure of which is totally incorporated herein by reference.

In U.S. Pat. No. 4,921,769, the disclosure of which is totally incorporated herein by reference, there are illustrated photoconductive imaging members with blocking layers of certain polyurethanes.

Illustrated in U.S. Pat. No. 5,473,064, the disclosure of which is totally incorporated herein by reference, is a process for the preparation of hydroxygallium phthalocyanine Type V, essentially free of chlorine.

Illustrated in U.S. Pat. No. 5,521,306, the disclosure of which is totally incorporated herein by reference, is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photogenerating pigments, which comprises hydrolyzing a gallium phthalocyanine precursor pigment by dissolving the hydroxygallium phthalocyanine in a strong acid, and then reprecipitating the resulting dissolved pigment in basic aqueous media; removing any ionic species formed by washing with water, concentrating the resulting aqueous slurry comprised of water and hydroxygallium phthalocyanine to a wet cake; removing water from said slurry by azeotropic distillation with an organic solvent, and subjecting said resulting pigment slurry to mixing with the addition of a second solvent to cause the formation of said hydroxygallium phthalocyanine polymorphs.

A number of photoconductors are disclosed in U.S. Pat. No. 5,489,496; U.S. Pat. No. 4,579,801; U.S. Pat. No. 4,518,669; U.S. Pat. No. 4,775,605; U.S. Pat. No. 5,656,407; U.S. Pat. No. 5,641,599; U.S. Pat. No. 5,344,734; U.S. Pat. No. 5,721,080; and U.S. Pat. No. 5,017,449, the entire disclosures

of which are totally incorporated herein by reference. Also, photoreceptors are disclosed in U.S. Pat. No. 6,200,716; U.S. Pat. No. 6,180,309; and U.S. Pat. No. 6,207,334, the entire disclosures of which are totally incorporated herein by reference.

A number of undercoat or charge blocking layers are disclosed in U.S. Pat. No. 4,464,450; U.S. Pat. No. 5,449,573; U.S. Pat. No. 5,385,796; and U.S. Pat. No. 5,928,824, the entire disclosures of which are totally incorporated herein by reference.

## SUMMARY

According to embodiments illustrated herein, and wherein ghosting is minimized or substantially eliminated, in images printed there are provided photoconductors that enable, it is believed, acceptable print quality in systems with high transfer current.

Embodiments disclosed herein also include a photoconductor comprising a substrate, a ground plane layer, and an undercoat layer as illustrated herein, disposed or deposited on the ground plane layer, especially a gold or gold containing ground plane, a photogenerating layer, and a charge transport layer formed on the photogenerating layer; a photoconductor comprised of a substrate, a ground plane layer, an undercoat layer disposed on the ground plane, wherein the undercoat layer comprises an aminosilane and a phosphonate, which primarily functions to provide for hole blocking of gold ground plane, minimization of CDS, excellent cyclic stability for the photoconductor, thus color stability for the xerographic prints.

## DETAILED DESCRIPTION

Aspects of the present disclosure relate to a photoconductor comprising a substrate; a ground plane layer; an undercoat layer thereover wherein the undercoat layer comprises an aminosilane and a phosphonate; a photogenerating layer; and at least one charge transport layer; a photoconductor comprising a substrate; a ground plane layer; an undercoat layer thereover comprised of a mixture of an aminosilane and a phosphonate; a photogenerating layer; and a charge transport layer; a rigid drum or flexible photoconductor comprising in sequence a supporting substrate; ground plane layer; a hole blocking layer comprised of an aminosilane and a phosphonate mixture; a photogenerating layer; and a charge transport layer, and wherein the phosphonate is selected from the group consisting of N,N-bis-(2-hydroxyethyl)aminomethane phosphonic acid diethyl ester, (methylthiomethyl)phosphonic acid diethyl ester, 2-hydroxyethylphosphonic acid dimethyl ester, cyanomethylphosphonic acid diethyl ester, di-n-butyl N,N-diethylcarbamoylmethylphosphonate, dibutyl N,N-diethylcarbamoylmethylphosphonate, diethyl(phthalimidomethyl)phosphonate, diethyl 1-pyrrolidinemethylphosphonate, diethyl 3,5-di-tert-butyl-4-hydroxybenzyl phosphonate, diphenyl(2,3-dihydro-2-thioxo-3-benzoxazolyl)phosphonate, monoethyl 3,5-di-tert-butyl-4-hydroxybenzylphosphonate, tetraethyl[4,4'-biphenylenebis(methylene)]bisphosphonate, diethyl 4-methoxyphenylphosphonate, tetraethyl [anthracene-9,10-diybis(methylene)]bisphosphonate, diethyl benzylphosphonate, bis(2,2,2-trifluoroethyl)(methoxycarbonylmethyl)phosphonate, diethyl phenacylphosphonate, diethyl(3-chlorobenzyl)phosphonate, diethyl cyanophosphonate, and diethyl phenylphosphonate; a photoconductor comprising a substrate; an undercoat layer thereover wherein the undercoat layer comprises an aminosilane and a phosphonate; a photogenerating layer; and at least

one charge transport layer, where at least one is, for example, from 1 to about 7, from 1 to about 5, from 1 to about 3, 1, or 2 layers; a photoconductor comprising a supporting substrate, a ground plane layer like gold; an undercoat layer thereover comprised of a mixture of an aminosilane and a phosphonate, a photogenerating layer, and a charge transport layer; a rigid drum or flexible belt photoconductor comprising in sequence a supporting substrate, such as a nonconductive substrate, thereover a ground plane layer; a hole blocking layer comprised of an aminosilane and a phosphonate, a photogenerating layer, and a charge transport layer; a photoconductive member or device comprising a substrate, a ground plane layer, the robust undercoat layer illustrated herein, and at least one imaging layer, such as a photogenerating layer and a charge transport layer or layers, formed on the undercoat layer; a photoconductor wherein the photogenerating layer is situated between the charge transport layer and the substrate, and which layer contains a resin binder; an electrophotographic imaging member which generally comprises at least a substrate layer, a ground plane layer, an undercoat layer, and where the undercoat layer is generally located between the substrate and deposited on the undercoat layer in sequence a photogenerating layer and a charge transport layer.

#### Ground Plane Layer Examples

In addition to gold or gold containing compounds, examples of ground plane layers are aluminum, titanium, titanium/zirconium, and other known compounds. The thickness of the metallic ground plane is from about 10 to about 100 nanometers. Specifically, the ground plane in embodiments is from about 20 to about 50, and more specifically, about 35 nanometers in thickness, and the titanium or titanium/zirconium ground plane is, for example, from about 10 to about 30, and more specifically, about 20 nanometers in thickness.

#### Undercoat Layer Component Examples

The undercoat layer in embodiments may be comprised of a number of suitable known components, in addition to the aminosilane and phosphonate mixture.

Phosphonate examples can be represented by the following structure/formula



wherein  $\text{R}_1$  is alkyl or aryl and derivatives thereof; and  $\text{R}_2$  and  $\text{R}_3$  are each independently hydrogen, an alkyl, or an aryl, and derivatives thereof. Examples of  $\text{R}_1$  include  $\text{N,N-bis-(2-hydroxyethyl)aminomethane}$ , methylthiomethyl, 2-hydroxyethyl, cyanomethyl,  $\text{N,N-diethylcarbamoylmethyl}$ ,  $\text{N,N-diethylcarbamoyl}$ , phthalimidomethyl, 1-pyrrolidinemethyl, 3,5-di-tert-butyl-4-hydroxybenzyl, 2,3-dihydro-2-thioxo-3-benzoxazolyl, 3,5-di-tert-butyl-4-hydroxybenzyl, 4-methoxyphenyl, benzyl, methoxycarbonylmethyl, phenacyl, 3-chlorobenzyl, phenyl, cyano, and the like. Examples of  $\text{R}_2$  and  $\text{R}_3$  include hydrogen, methyl, ethyl, propyl, isopropyl, n-butyl, isobutyl, phenyl, 2,2,2-trifluoroethyl and the like.

Specific phosphonate examples include  $\text{N,N-bis-(2-hydroxyethyl)aminomethanephosphonic acid diethyl ester}$ ,

(methylthiomethyl)phosphonic acid diethyl ester, 2-hydroxyethylphosphonic acid dimethyl ester, cyanomethylphosphonic acid diethyl ester, di-n-butyl  $\text{N,N-diethylcarbamoyl}$  methylphosphonate, dibutyl  $\text{N,N-diethylcarbamoylphosphonate}$ , diethyl(phthalimidomethyl)phosphonate, diethyl 1-pyrrolidinemethylphosphonate, diethyl 3,5-di-tert-butyl-4-hydroxybenzylphosphonate, diphenyl(2,3-dihydro-2-thioxo-3-benzoxazolyl)phosphonate, monoethyl 3,5-di-tert-butyl-4-hydroxybenzylphosphonate, tetraethyl[4,4'-biphenylenebis(methylene)]bisphosphonate, diethyl 4-methoxyphenylphosphonate, tetraethyl [anthracene-9,10-diybis(methylene)]bisphosphonate, diethyl benzylphosphonate, bis(2,2,2-trifluoroethyl)(methoxycarbonylmethyl)phosphonate, diethyl phenacylphosphonate, diethyl(3-chlorobenzyl)phosphonate, diethyl cyano-phosphonate, diethyl phenylphosphonate, and the like.

In embodiments, the phosphonate present in the undercoat layer is represented by at least one of the following formulas/structures



9



Aminosilane examples included in the hole blocking layer can be represented by the following structure/formula



wherein  $R_1$  is an alkylene group containing, for example, from 1 to about 25 carbon atoms;  $R_2$  and  $R_3$  are independently selected from the group consisting of at least one of hydrogen, alkyl containing, for example, from 1 to about 5, and more specifically, about 3 carbon atoms; an aryl with, for example, from about 6 to about 36 carbon atoms, such as a phenyl group

10

and a poly(alkylene like ethylene amino) group; and  $R_4$ ,  $R_5$ , and  $R_6$  are independently selected from an alkyl group containing, for example, from 1 to about 6, and more specifically, about 4 carbon atoms.

- 5 Aminosilane specific examples include 3-aminopropyl triethoxysilane, N,N-dimethyl-3-aminopropyl triethoxysilane, N-phenylaminopropyl trimethoxysilane, triethoxysilylpropylethylene diamine, trimethoxysilylpropylethylene diamine, trimethoxysilylpropyl diethylene triamine, N-ami-  
10 noethyl-3-aminopropyl trimethoxysilane, N-2-aminoethyl-3-aminopropyl trimethoxysilane, N-2-aminoethyl-3-amino- propyl tris(ethylethoxy)silane, p-aminophenyl trimethoxysilane, N,N'-dimethyl-3-aminopropyl triethoxysilane, 3-aminopropylmethyl diethoxysilane, 3-aminopropyl trimethoxysilane, N-methylaminopropyl triethoxysilane, methyl[2-(3-trimethoxysilylpropylamino)ethylamino]-3- propionate, (N,N'-dimethyl 3-amino)propyl triethoxysilane, N,N-dimethylaminophenyl triethoxysilane, trimethoxysilylpropyl diethylene triamine, and the like, and mixtures thereof.  
15  
20 Yet more specific aminosilane materials are 3-aminopropyl triethoxysilane ( $\gamma$ -APS), N-aminoethyl-3-aminopropyl triethoxysilane, (N,N'-dimethyl-3-amino)propyl triethoxysilane, and mixtures thereof.

The aminosilane may be hydrolyzed to form a hydrolyzed silane solution before being added into the final undercoat coating solution or dispersion. During hydrolysis of the aminosilanes, the hydrolyzable groups, such as alkoxy groups, are replaced with hydroxyl groups. The pH of the hydrolyzed silane solution can be controlled to obtain excellent characteristics on curing, and to result in electrical stability. A solution pH of, for example, from about 4 to about 10 can be selected, and more specifically, a pH of from about 7 to about 8. Control of the pH of the hydrolyzed silane solution may be affected with any suitable material, such as generally organic or inorganic acids. Typical organic and inorganic acids include acetic acid, citric acid, formic acid, hydrogen iodide, phosphoric acid, hydrofluorosilicic acid, p-toluenesulfonic acid, and the like.

Various amounts of the phosphonate can be included in the

- 40 hole blocking layer, such as, for example, from about 0.1 to about 50, from about 1 to about 40, or from about 5 to about 30, with the amount of aminosilane being, for example, from about 50 to about 99.9 weight percent, from about 60 to about 99, or from about 70 to about 95 weight percent; and where  
45 the total of the two components is equal to about 100 percent. The hole blocking layer thickness can be of any suitable value, such as for example, from about 0.01 to about 1 micron, from about 0.02 to about 0.5 micron, from about 0.03 to about 0.2 micron.

50 There can be further included in the undercoat or hole blocking layer a number of polymer binders, for example polyacetal resins such as polyvinyl butyral resins, aminoplast resins such as melamine resins or mixtures of these resins, and which resins or mixtures of resins function primarily to

55 disperse mixture of the aminosilane and the phosphonate, and other known suitable components that may be present in the undercoat.

## Polymer Binder Examples

- 60 In embodiments, an aminoplast resin may be selected as a component for the undercoat layer. Aminoplast resin refers, for example, to a type of amino resin generated from a nitrogen-containing substance, and formaldehyde wherein the nitrogen-containing substance includes, for example, melamine, urea, benzoguanamine, and glycoluril. Undercoat layer binders also include melamine resins are considered

## 11

amino resins prepared from melamine and formaldehyde. Melamine resins are known under various trade names, including but not limited to CYMEL®, BEETLE™, DYNOMINT™, BECKAMINETM, UFRT™, BAKELITE™, ISOMINT™, MELAICART™, MELBRITE™, MELMEX™, MELOPAST™, RESART™, and ULTRAPAST™. As used herein, urea resins are amino resins made from urea and formaldehyde. Urea resins are known under various trade names, including but not limited to CYMEL®, BEETLE™, UFRM™, DYNOMINT™, BECKAMINETM, and AMIREMETM.

In various embodiments, the melamine resin can be represented by



wherein R<sub>1</sub>, R<sub>2</sub>, R<sub>3</sub>, R<sub>4</sub>, R<sub>5</sub> and R<sub>6</sub> each independently represents a hydrogen atom or an alkyl chain with, for example, from 1 to about 8 carbon atoms, and more specifically, from 1 to about 4 carbon atoms. In embodiments, the melamine resin is water-soluble, dispersible or nondispersible. Specific examples of melamine resins include highly alkylated/alkoxylated, partially alkylated/alkoxylated, or mixed alkylated/alkoxylated; methylated, n-butylated or isobutylated; highly methylated melamine resins such as CYMEL® 350, 9370; methylated high imino melamine resins (partially methylolated and highly alkylated) such as CYMEL® 323, 327; partially methylated melamine resins (highly methylolated and partially methylated) such as CYMEL® 373, 370; high solids mixed ether melamine resins such as CYMEL® 1130, 324; n-butylated melamine resins such as CYMEL® 1151, 615; n-butylated high imino melamine resins such as CYMEL® 1158; and iso-butylated melamine resins such as CYMEL® 255-10. CYMEL® melamine resins are commercially available from CYTEC Industries, Inc., and yet more specifically, the melamine resin may be selected from the group consisting of methylated formaldehyde-melamine resin, methoxymethylated melamine resin, ethoxymethylated melamine resin, propoxymethylated melamine resin, butoxymethylated melamine resin, hexamethylol melamine resin, alkoxyalkylated melamine resins such as methoxymethylated melamine resin, ethoxymethylated melamine resin, propoxymethylated melamine resin, butoxymethylated melamine resin, and mixtures thereof.

Undercoat layer urea resin binder examples can be represented by



## 12

wherein R<sub>1</sub>, R<sub>2</sub>, R<sub>3</sub>, and R<sub>4</sub> each independently represents a hydrogen atom, an alkyl chain with, for example, from 1 to about 8 carbon atoms, or with 1 to 4 carbon atoms, and which urea resin can be water soluble, dispersible, or indispersible.

The urea resin can be a highly alkylated/alkoxylated, partially alkylated/alkoxylated, or mixed alkylated/alkoxylated, and more specifically, the urea resin is a methylated, n-butylated, or isobutylated polymer. Specific examples of the urea resin include methylated urea resins such as CYMEL® U-65, 10 U-382; n-butylated urea resins such as CYMEL® U-1054, UB-30-B; or isobutylated urea resins such as CYMEL® U-662, UI-19-I. CYMEL® urea resins are commercially available from CYTEC Industries, Inc.

Undercoat layer examples of benzoguanamine binder resins can be represented by



wherein R<sub>1</sub>, R<sub>2</sub>, R<sub>3</sub>, and R<sub>4</sub> each independently represents a hydrogen atom or an alkyl chain as illustrated herein. In embodiments, the benzoguanamine resin is water soluble, dispersible, or indispersible. The benzoguanamine resin can be highly alkylated/alkoxylated, partially alkylated/alkoxylated, or a mixed alkylated/alkoxylated material. Specific examples of the benzoguanamine resin include methylated, n-butylated, or isobutylated, with examples of the benzoguanamine resin being CYMEL® 659, 5010, 5011. CYMEL® benzoguanamine resins are commercially available from CYTEC Industries, Inc. Benzoguanamine resin examples can be generally comprised of amino resins generated from benzoguanamine, and formaldehyde. Benzoguanamine resins are known under various trade names, including but not limited to CYMEL®, BEETLE™, and UFORMITE™. Glycoluril resins are amino resins obtained from glycoluril and formaldehyde, and are known under various trade names, including but not limited to CYMEL®, and POWDER-LINK™. The aminoplast resins can be highly alkylated or partially alkylated.

Glycoluril resin undercoat binder examples are



wherein R<sub>1</sub>, R<sub>2</sub>, R<sub>3</sub>, and R<sub>4</sub> each independently represents a hydrogen atom or an alkyl chain as illustrated herein with, for example, 1 to about 8 carbon atoms, or with 1 to about 4 carbon atoms. The glycoluril resin can be water soluble,

dispersible, or indispersible. Examples of the glycoluril resin include highly alkylated/alkoxylated, partially alkylated/alkoxylated, or mixed alkylated/alkoxylated, and more specifically, the glycoluril resin can be methylated, n-butylated, or isobutylated. Specific examples of the glycoluril resin include CYMEL® 1170, 1171. CYMEL® glycoluril resins are commercially available from CYTEC Industries, Inc.

In embodiments, polyacetal resin hole blocking or under-coat layer binders include polyvinyl butyral formed by the well-known reactions between aldehydes and alcohols. The addition of one molecule of an alcohol to one molecule of an aldehyde produces a hemiacetal. Hemiacetals are rarely isolated because of their inherent instability, but rather are further reacted with another molecule of alcohol to form a stable acetal. Polyvinyl acetals are prepared from aldehydes and polyvinyl alcohols. Polyvinyl alcohols are high molecular weight resins containing various percentages of hydroxyl and acetate groups produced by hydrolysis of polyvinyl acetate. The conditions of the acetal reaction and the concentration of the particular aldehyde and polyvinyl alcohol used are controlled to form polymers containing predetermined proportions of hydroxyl groups, acetate groups, and acetal groups. The polyvinyl butyral can be represented by



The proportions of polyvinyl butyral (A), polyvinyl alcohol (B), and polyvinyl acetate (C) are controlled, and they are randomly distributed along the molecule. The mole percent of polyvinyl butyral (A) is from about 50 to about 95, that of polyvinyl alcohol (B) is from about 5 to about 30, and that of polyvinyl acetate (C) is from about 0 to about 10. In addition to vinyl butyral (A), other vinyl acetals can be optionally present in the molecule including vinyl isobutyral (D), vinyl propyral (E), vinyl acetacetal (F), and vinyl formal (G). The total mole percent of all the monomeric units in one molecule is about 100.

Examples of hole blocking layer polyvinyl butyral include BUTVARTM B-72 ( $M_w$ =170,000 to 250,000, A=80, B=17.5 to 20, C=0 to 2.5), B-74 ( $M_w$ =120,000 to 150,000, A=80, B=17.5 to 20, C=0 to 2.5), B-76 ( $M_w$ =90,000 to 120,000, A=88, B=11 to 13, C=0 to 1.5), B-79 ( $M_w$ =50,000 to 80,000, A=88, B=10.5 to 13, C=0 to 1.5), B-90 ( $M_w$ =70,000 to 100,000, A=80, B=18 to 20, C=0 to 1.5), and B-98 ( $M_w$ =40,000 to 70,000, A=80, B=18 to 20, C=0 to 2.5), all commercially available from Solutia, St. Louis, Mo.; S-LECTM BL-1 (degree of polymerization=300, A=63±3, B=37, C=3), BM-1 (degree of polymerization=650, A=65±3, B=32, C=3), BM-S (degree of polymerization=850, A>70, B=25, C=4 to 6), BX-2 (degree of polymerization=1,700, A=45, B=33, G=20), all commercially available from Sekisui Chemical Co., Ltd., Tokyo, Japan.

The hole blocking layer can contain a single resin binder, a mixture of resin binders, such as from 2 to about 7, and the like, and where for the mixtures the percentage amounts selected for each resin varies providing that the mixture contains about 100 percent by weight of the first and second resin, or the first, second, and third resin.

In embodiments, the undercoat layer may contain various colorants such as organic pigments and organic dyes, including, but not limited to, azo pigments, quinoline pigments, perylene pigments, indigo pigments, thiocindigo pigments, 5 bisbenzimidazole pigments, phthalocyanine pigments, quinacridone pigments, quinoline pigments, lake pigments, azo lake pigments, anthraquinone pigments, oxazine pigments, dioxazine pigments, triphenylmethane pigments, azulenium dyes, squalium dyes, pyrylium dyes, triallylmethane 10 dyes, xanthene dyes, thiiazine dyes, and cyanine dyes. In various embodiments, the undercoat layer may include inorganic materials, such as amorphous silicon, amorphous selenium, tellurium, a selenium-tellurium alloy, cadmium sulfide, antimony sulfide, titanium oxide, tin oxide, zinc oxide, and 15 zinc sulfide, and mixtures thereof. The colorant can be selected in various suitable amounts like from about 0.5 to about 20 weight percent, and more specifically, from 1 to about 12 weight percent.

about 12 weight percent.

The hole blocking layer can, in embodiments, be prepared by a number of known methods, the process parameters being dependent, for example, on the photoconductor member desired. The hole blocking layer can be coated as a solution or a dispersion onto the ground plane layer by the use of a spray coater, dip coater, extrusion coater, roller coater, wire-bar coater, slot coater, doctor blade coater, gravure coater, and the like, and dried at from about 40° C. to about 200° C. for a suitable period of time, such as from about 1 minute to about 10 hours, under stationary conditions or in an air flow. The coating can be accomplished to provide a final coating thickness of from about 0.01 to about 1 micron, or from about 0.02 to about 0.5 micron after drying.

## Photoconductor Layer Examples

35 The thickness of the photoconductive substrate layer depends on many factors including economical considerations, electrical characteristics, and the like; thus, this layer may be of a substantial thickness, for example over 3,000 microns, such as from about 500 to about 2,000, from about 40 300 to about 700 microns, or of a minimum thickness. In embodiments, the thickness of this layer is from about 75 microns to about 300 microns, or from about 100 to about 150 microns.

The substrate may be opaque, substantially transparent, or be of a number of other suitable known forms and may comprise any suitable material having the required mechanical properties. Accordingly, the substrate may comprise a layer of an electrically nonconductive or conductive material such as an inorganic or an organic composition. As electrically nonconducting materials, there may be employed various resins known for this purpose including polyesters, polycarbonates, polyamides, polyurethanes, and the like, which are flexible as thin webs. An electrically conducting substrate may be any suitable metal of, for example, aluminum, nickel, steel, copper, and the like, or a polymeric material, as described above, filled with an electrically conducting substance, such as carbon, metallic powder, and the like, or an organic electrically conducting material. The electrically insulating or conductive substrate may be in the form of an endless flexible belt, a web, a rigid cylinder, a sheet, and the like. The thickness of the substrate layer depends on numerous factors including strength desired and economical considerations. For a drum, as disclosed in a copending application referenced herein, this layer may be of a substantial thickness of, for example, up to many centimeters or of a minimum thickness of less than a millimeter. Similarly, a flexible belt may be of substantial thickness of, for example,

about 250 micrometers, or of minimum thickness of less than about 50 micrometers, provided there are no adverse effects on the final electrophotographic device. In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors.

Illustrative examples of substrates are as illustrated herein, and more specifically, substrates selected for the imaging members of the present disclosure, and which substrates can be opaque or substantially transparent comprise a layer of insulating material including inorganic or organic polymeric materials, such as MYLAR® a commercially available polymer, MYLAR® containing titanium, a layer of an organic or inorganic material having a semiconductive surface layer, such as indium tin oxide, or aluminum arranged thereon, or a conductive material inclusive of aluminum, chromium, nickel, brass, or the like. The substrate may be flexible, seamless, or rigid, and may have a number of many different configurations, such as for example, a plate, a cylindrical drum, a scroll, an endless flexible belt, and the like. In embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

The photogenerating layer in embodiments is comprised of, for example, a number of known photogenerating pigments including, for example, Type V hydroxygallium phthalocyanine, Type IV or V titanyl phthalocyanine or chlorogallium phthalocyanine, and a resin binder like poly(vinyl chloride-co-vinyl acetate) copolymer, such as VMCH (available from Dow Chemical), or polycarbonate. Generally, the photogenerating layer can contain known photogenerating pigments, such as metal phthalocyanines, metal free phthalocyanines, alkylhydroxygallium phthalocyanines, hydroxygallium phthalocyanines, chlorogallium phthalocyanines, perylenes, especially bis(benzimidazo)perylene, titanyl phthalocyanines, and the like, and more specifically, vanadyl phthalocyanines, Type V hydroxygallium phthalocyanines, and inorganic components such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerating layer depends on a number of factors, including the thicknesses of the other layers, and the amount of photogenerating material contained in the photogenerating layer. Accordingly, this layer can be of a thickness of, for example, from about 0.05 micron to about 10 microns, and more specifically, from about 0.25 micron to about 2 microns when, for example, the photogenerating compositions are present in an amount of from about 30 to about 75 percent by volume. The maximum thickness of this layer in embodiments is dependent primarily upon factors, such as photosensitivity, electrical properties and mechanical considerations. The photogenerating layer binder resin is present in various suitable amounts of, for example, from about 1 to about 50, and more specifically, from about 1 to about 10 weight percent, and which resin may be selected from a number of known polymers, such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alco-

hol), polyacrylonitrile, polystyrene, and the like. It is desirable to select a coating solvent that does not substantially disturb or adversely affect the other previously coated layers of the device. Generally, however, from about 5 percent by volume to about 90 percent by volume of the photogenerating pigment is dispersed in about 10 percent by volume to about 95 percent by volume of the resinous binder, or from about 20 percent by volume to about 30 percent by volume of the photogenerating pigment is dispersed in about 70 percent by volume to about 80 percent by volume of the resinous binder composition. In one embodiment, about 8 percent by volume of the photogenerating pigment is dispersed in about 92 percent by volume of the resinous binder composition. Examples of coating solvents for the photogenerating layer are ketones, alcohols, aromatic hydrocarbons, halogenated aliphatic hydrocarbons, ethers, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The photogenerating layer may comprise amorphous films of selenium and alloys of selenium and arsenic, tellurium, germanium, and the like, hydrogenated amorphous silicone and compounds of silicone and germanium, carbon, oxygen, nitrogen, and the like fabricated by vacuum evaporation or deposition. The photogenerating layer may also comprise inorganic pigments of crystalline selenium and its alloys; Groups II to VI compounds; and organic pigments such as quinacridones, polycyclic pigments such as dibromo anthranthrone pigments, perylene and perinone diamines, polynuclear aromatic quinones, azo pigments including bis-, tris- and tetrakis-azos, and the like dispersed in a film forming polymeric binder and fabricated by solvent coating techniques.

Examples of polymeric binder materials that can be selected as the matrix for the photogenerating layer components are thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, poly(vinyl chloride), vinyl chloride and vinyl acetate copolymers, acrylate copolymers, alkyd resins, cellulosic film formers, poly(amideimide), styrene-butadiene copolymers, vinylidene chloride-vinyl chloride copolymers, vinyl acetate-vinylidene chloride copolymers, styrene-alkyd resins, poly(vinyl carbazole), and the like. These polymers may be block, random, or alternating copolymers.

Various suitable and conventional known processes may be selected to mix, and thereafter apply the photogenerating layer coating mixture to the substrate, and more specifically, to the hole blocking layer or other layers like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like. The coating of the photogenerating layer on the UCL (undercoat layer) in

embodiments of the present disclosure can be accomplished such that the final dry thickness of the photogenerating layer is as illustrated herein, and can be, for example, from about 0.01 to about 30 microns after being dried at, for example, about 40° C. to about 150° C. for about 1 to about 90 minutes. More specifically, a photogenerating layer of a thickness, for example, of from about 0.1 to about 30, or from about 0.5 to about 2 microns can be applied to or deposited on the substrate, on other surfaces in between the substrate and the charge transport layer, and the like. The hole blocking layer or UCL may be applied to the ground plane layer prior to the application of a photogenerating layer.

A suitable known adhesive layer can be included in the photoconductor. Typical adhesive layer materials include, for example, polyesters, polyurethanes, and the like. The adhesive layer thickness can vary, and in embodiments is, for example, from about 0.05 micrometer (500 Angstroms) to about 0.3 micrometer (3,000 Angstroms). The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying, and the like. As optional adhesive layers usually in contact with or situated between the hole blocking layer and the photogenerating layer, there can be selected various known substances inclusive of copolymers, polyamides, poly(vinyl butyral), poly(vinyl alcohol), polyurethane, and polyacrylonitrile. This layer is, for example, of a thickness of from about 0.001 micron to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicone nitride, carbon black, and the like, to provide, for example, in embodiments of the present disclosure, further desirable electrical and optical properties.

A number of charge transport materials, especially known hole transport molecules, may be selected for the charge transport layer, examples of which are aryl amines of the formulas/structures, and which layer is generally of a thickness of from about 5 microns to about 75 microns, and more specifically, of a thickness of from about 10 microns to about 40 microns



wherein X is a suitable hydrocarbon like alkyl, alkoxy, and aryl; a halogen, or mixtures thereof, and especially those substituents selected from the group consisting of Cl and CH<sub>3</sub>; and molecules of the following formulas



wherein X, Y and Z are a suitable substituent like a hydrocarbon, such as independently alkyl, alkoxy, or aryl; a halogen, or mixtures thereof, and wherein at least one of Y or Z is present. Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide, and fluoride. Substituted alkyls, alkoxy, and aryls can also be selected in embodiments. At least one charge transport refers, for example, to 1, from 1 to about 7, from 1 to about 4, and from 1 to about 2.

Examples of specific aryl amines include N,N'-diphenyl-N,N'-bis(alkylphenyl)-1,1-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, N,N'-diphenyl-N,N'-bis(3-chlorophenyl)-[p-terphenyl]-4,4'-diamine, and the like. Other known charge transport layer molecules can be selected, reference for example, U.S. Pat. Nos. 4,921,773 and 4,464,450, the disclosures of which are totally incorporated herein by reference.

Examples of the binder materials selected for the charge transport layer or layers include polycarbonates, polyarylates, acrylate polymers, vinyl polymers, cellulose polymers, polyesters, polysiloxanes, polyamides, polyurethanes, poly(cyclo olefins), epoxies, and random or alternating copolymers thereof; and more specifically, polycarbonates such as poly(4,4'-isopropylidene-diphenylene)carbonate (also referred to as bisphenol-A-polycarbonate), poly(4,4'-cyclohexylidinediphenylene)carbonate (also referred to as bisphenol-Z-polycarbonate), poly(4,4'-isopropylidene-3,3'-dimethyl-diphenyl)carbonate (also referred to as bisphenol-C-polycarbonate), and the like. In embodiments, electrically inactive binders are comprised of polycarbonate resins with a molecular weight of from about 20,000 to about 100,000, or with a molecular weight M<sub>w</sub> of from about 50,000 to about 100,000 preferred. Generally, the transport layer contains from about 10 to about 75 percent by weight of the charge

transport material, and more specifically, from about 35 percent to about 50 percent of this material.

The charge transport layer or layers, and more specifically, a first charge transport in contact with the photogenerating layer, and thereover a top or second charge transport overcoating layer may comprise charge transporting small molecules dissolved or molecularly dispersed in a film forming electrically inert polymer such as a polycarbonate. In embodiments, "dissolved" refers, for example, to forming a solution in which the small molecule is dissolved in the polymer to form a homogeneous phase; and "molecularly dispersed in embodiments" refers, for example, to charge transporting molecules dispersed in the polymer, the small molecules being dispersed in the polymer on a molecular scale. Various charge transporting or electrically active small molecules may be selected for the charge transport layer or layers. In embodiments, charge transport refers, for example, to charge transporting molecules as a monomer that allows the free charge generated in the photogenerating layer to be transported across the transport layer.

Examples of hole transporting molecules selected for the charge transport layer or layers, and present in various effective amounts include, for example, pyrazolines such as 1-phenyl-3-(4'-diethylamino styryl)-5-(4"-diethylamino phenyl) pyrazoline; aryl amines such as N,N'-diphenyl-N,N'-bis(3-methylphenyl)-(1,1-biphenyl)-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-NR-bis-(4-isopropylphenyl)-[p-terphenyl]-4,4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4"-diamine, and N,N'-diphenyl-N,N'-bis(3-chlorophenyl)-[p-terphenyl]-4,4'-diamine; hydrazones such as N-phenyl-N-methyl-3-(9-ethyl) carbazyl hydrazone, and 4-diethyl amino benzaldehyde-1,2-diphenyl hydrazone; and oxadiazoles such as 2,5-bis(4,N,N-diethylaminophenyl)-1,2,4-oxadiazole, stilbenes, and the like. A small molecule charge transporting compound that permits injection of holes into the photogenerating layer with high efficiency, and transports them across the charge transport layer with short transit times includes N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, and N,N'-diphenyl-N,N'-bis(3-chlorophenyl)-[p-terphenyl]-4,4'-diamine, or mixtures thereof. If desired, the charge transport material in the charge transport layer may comprise a polymeric charge transport material or a combination of a small molecule charge transport material and a polymeric charge transport material.

Examples of components or materials optionally incorporated into the charge transport layers or at least one charge transport layer to, for example, enable improved lateral charge migration (LCM) resistance include hindered phenolic antioxidants, such as tetrakis methylene(3,5-di-tert-butyl-4-hydroxy hydrocinnamate)methane (IRGANOX™ 1010, available from Ciba Specialty Chemical), butylated hydroxytoluene (BHT), and other hindered phenolic antioxidants including SUMILIZER™ BHT-R, MDP-S, BBM-S,

WX-R, NW, BP-76, BP-101, GA-80, GM and GS (available from Sumitomo Chemical Co., Ltd.), IRGANOX™ 1035, 1076, 1098, 1135, 1141, 1222, 1330, 1425WL, 1520L, 245, 259, 3114, 3790, 5057 and 565 (available from Ciba Specialties Chemicals), and ADEKA STAB™ AO-20, AO-30, AO-40, AO-50, AO-60, AO-70, AO-80 and AO-330 (available from Asahi Denka Co., Ltd.); hindered amine antioxidants such as SANOL™ LS-2626, LS-765, LS-770 and LS-744 (available from SNKYO CO., Ltd.), TINUVIN™ 144 and 622LD (available from Ciba Specialties Chemicals), MARK™ LA57, LA67, LA62, LA68 and LA63 (available from Asahi Denka Co., Ltd.), and SUMILIZER™ TPS (available from Sumitomo Chemical Co., Ltd.); thioether antioxidants such as SUMILIZER™ TP-D (available from Sumitomo Chemical Co., Ltd.); phosphite antioxidants such as MARK™ 2112, PEP-8, PEP-24G, PEP-36, 329K and HP-10 (available from Asahi Denka Co., Ltd.); other molecules such as bis(4-diethylamino-2-methylphenyl)phenylmethane (BDETPM), bis-[2-methyl-4-(N-2-hydroxyethyl-N-ethylaminophenyl)]-phenylmethane (DHTPM), and the like. The weight percent of the antioxidant in at least one of the charge transport layers is from about 0 to about 20, from about 1 to about 10, or from about 3 to about 8 weight percent.

A number of processes may be used to mix, and thereafter apply the charge transport layer or layers coating mixture to the photogenerating layer. Typical application techniques include spraying, dip coating, and roll coating, wire wound rod coating, and the like. Drying of the charge transport deposited coating may be effected by any suitable conventional technique such as oven drying, infrared radiation drying, air drying, and the like.

The thickness of each of the charge transport layers in embodiments is, for example, from about 10 to about 75, from about 15 to about 50 micrometers, but thicknesses outside these ranges may in embodiments also be selected. The charge transport layer should be an insulator to the extent that an electrostatic charge placed on the hole transport layer is not conducted in the absence of illumination at a rate sufficient to prevent formation and retention of an electrostatic latent image thereon. In general, the ratio of the thickness of the charge transport layer to the photogenerating layer can be from about 2:1 to about 200:1, and in some instances 400:1. The charge transport layer is substantially nonabsorbing to visible light or radiation in the region of intended use, but is electrically "active" in that it allows the injection of photogenerated holes from the photoconductive layer or photogenerating layer, and allows these holes to be transported to selectively discharge a surface charge on the surface of the active layer.

The thickness of the continuous charge transport layer selected depends upon the abrasiveness of the charging (bias charging roll), cleaning (blade or web), development (brush), transfer (bias transfer roll), and the like in the system employed, and can be up to about 10 micrometers. In embodiments, the thickness for each charge transport layer can be, for example, from about 1 micrometer to about 5 micrometers. Various suitable and conventional methods may be used to mix, and thereafter apply an overcoat top charge transport layer coating mixture to the photoconductor. Typical application techniques include spraying, dip coating, roll coating, wire wound rod coating, and the like. Drying of the deposited coating may be effected by any suitable conventional technique, such as oven drying, infrared radiation drying, air drying, and the like. The dried overcoat layer of this disclosure should transport holes during imaging, and should not have too high a free carrier concentration. Free carrier concentration in the overcoat increases the dark decay.

21

The following Examples are provided. All proportions are by weight unless otherwise indicated.

#### Comparative Example 1

A ground plane layer of zirconium/titanium was prepared by vacuum sputtering or vacuum evaporation of a 0.02 micron thick zirconium/titanium metal layer onto a biaxially oriented polyethylene naphthalate substrate (KALEDEX™ 2000) having a thickness of 3.5 mils.

Subsequently, there was applied thereon, with a gravure applicator or an extrusion coater, a hole blocking layer solution containing 50 grams of 3-aminopropyl triethoxysilane ( $\gamma$ -APS), 41.2 grams of water, 15 grams of acetic acid, 684.8 grams of denatured alcohol, and 200 grams of heptane. This layer was then dried for about 1 minute at 120° C. in a forced air dryer. The resulting hole blocking layer had a dry thickness of 0.04 micron. An adhesive layer was then deposited by applying a wet coating over the blocking layer, using a gravure applicator or an extrusion coater, and which adhesive contained 0.2 percent by weight based on the total weight of the solution of the copolyester adhesive (ARDEL D100™ available from Toyota Hsutsu Inc.) in a 60:30:10 volume ratio mixture of tetrahydrofuran/monochlorobenzene/methylene chloride. The adhesive layer was then dried for about 1 minute at 120° C. in the forced air dryer of the coater. The resulting adhesive layer had a dry thickness of 0.02 micron.

A photogenerating layer dispersion was prepared by introducing 0.45 gram of the known polycarbonate IUPILON 200™ (PCZ-200) weight average molecular weight of 20,000, available from Mitsubishi Gas Chemical Corporation, and 50 milliliters of tetrahydrofuran into a 4 ounce glass bottle. To this solution were added 2.4 grams of hydroxygallium phthalocyanine and 300 grams of  $\frac{1}{8}$  inch (3.2 millimeters) diameter stainless steel shot. This mixture was then placed on a ball mill for 8 hours. Subsequently, 2.25 grams of PCZ-200 were dissolved in 46.1 grams of tetrahydrofuran, and added to the hydroxygallium phthalocyanine dispersion. This slurry was then placed on a shaker for 10 minutes. The resulting dispersion was, thereafter, applied to the above adhesive interface with a Bird applicator to form a photogenerating layer having a wet thickness of 0.50 mil. The photogenerating layer was dried at 120° C. for 1 minute in a forced air oven to form a dry photogenerating layer having a thickness of 0.8 micron.

(A) The photogenerating layer was then coated with a single charge transport layer prepared by introducing into an amber glass bottle in a weight ratio of 50/50, N,N'-bis(methylphenyl)-1,1-biphenyl-4,4'-diamine (TBD) and poly(4,4'-isopropylidene diphenyl)carbonate, a known bisphenol A polycarbonate having a  $M_w$  molecular weight average of about 120,000, commercially available from Farbenfabriken Bayer A.G. as MAKROLON® 5705. The resulting mixture was then dissolved in methylene chloride to form a solution containing 15.6 percent by weight solids. This solution was applied on the photogenerating layer to form the charge transport layer coating that upon drying (120° C. for 1 minute) had a thickness of 29 microns. During this coating process, the humidity was equal to or less than 30 percent, for example 25 percent.

(B) In another embodiment, the resulting photogenerating layer was then coated with a dual charge transport layer. The first charge transport layer was prepared by introducing into an amber glass bottle in a weight ratio of 50/50, N,N'-bis(methylphenyl)-1,1-biphenyl-4,4'-diamine (TBD) and poly(4,4'-isopropylidene diphenyl)carbonate, a known bisphenol A polycarbonate having a  $M_w$  molecular weight average of

22

about 120,000, commercially available from Farbenfabriken Bayer A.G. as MAKROLON® 5705. The resulting mixture was then dissolved in methylene chloride to form a solution containing 15.6 percent by weight solids. This solution was applied on the photogenerating layer to form the charge transport layer coating that upon drying (120° C. for 1 minute) had a thickness of 14.5 microns. During this coating process, the humidity was equal to or less than 30 percent, for example 25 percent.

10 The above first pass charge transport layer (CTL) was then overcoated with a second top charge transport layer in a second pass. The charge transport layer solution of the top layer was prepared by introducing into an amber glass bottle in a weight ratio of 0.35:0.65 N,N'-diphenyl-N,N'-bis(3-methylphenyl)-1,1'-biphenyl-4,4'-diamine, and MAKROLON® 5705, a known polycarbonate resin having a molecular weight average of from about 50,000 to about 100,000, commercially available from Farbenfabriken Bayer A.G. The resulting mixture was then dissolved in methylene chloride to form a solution containing 15 percent by weight solids. This solution was applied, using a 2 mil Bird bar, on the bottom layer of the charge transport layer to form a coating that upon drying (120° C. for 1 minute) had a thickness of 14.5 microns. During this coating process, the humidity was equal to or less than 15 percent. The total two-layer CTL thickness was 29 microns.

#### Comparative Example 2

30 Two photoconductors 2 (A) and 2(B) were prepared by repeating the above process of Comparative Example 1(A) and (B) above, except in place of the zirconium/titanium ground plane, there was selected a 0.035 micron gold ground plane deposited onto a biaxially oriented polyethylene naphthalate substrate (KALEDEX™ 2000) having a thickness of 3.5 mils via vacuum sputtering or vacuum evaporation.

#### Example I

40 A photoconductor was prepared by repeating the process of Comparative Example 2(A) except that the hole blocking layer solution was prepared by further adding to the hole blocking layer solution 10 weight percent of N,N-bis-(2-hydroxylethyl)aminomethane phosphonic acid diethyl ester, and the resulting hole blocking layer of a thickness of 0.04 micron was coated and dried (120° C./1 minute) on the gold ground plane (0.035 micron).

#### Example II

50 A photoconductor was prepared by repeating the process of Comparative Example 2(A) except that the hole blocking layer solution was prepared by further adding to the hole blocking layer solution 20 weight percent of diethyl(phthalimidomethyl)phosphonate, and the resulting hole blocking layer of a thickness of 0.04 micron was coated and dried (120° C./1 minute) on the gold ground plane (0.035 micron).

#### Example III

60 A number of photoconductors are prepared by repeating the process of Examples I and II except that the hole blocking layer could include, in place of N,N-bis-(2-hydroxylethyl)aminomethane phosphonic acid diethyl ester or diethyl(phthalimidomethyl)phosphonate, 10 weight percent of (methylthiomethyl)phosphonic acid diethyl ester, 2-hydroxyethylphosphonic acid dimethyl ester, cyanometh-

ylphosphonic acid diethyl ester, di-n-butyl N,N-diethylcarbamoyl methylphosphonate, dibutyl N,N-diethylcarbamoylphosphonate, diethyl 1-pyrrolidinemethylphosphonate, diethyl 3,5-di-tert-butyl-4-hydroxybenzyl phosphonate, diphenyl(2,3-dihydro-2-thioxo-3-benzoxazolyl)phosphonate, monoethyl 3,5-di-tert-butyl-4-hydroxybenzylphosphonate, tetraethyl[4,4'-biphenyl]enebis(methylene)]bisphosphonate, diethyl 4-methoxyphenyl phosphonate, tetraethyl [anthracene-9,10-diyl]bis(methylene)]bisphosphonate, diethyl benzylphosphonate, bis(2,2,2-trifluoroethyl)(methoxycarbonylmethyl)phosphonate, diethyl phenacylphosphonate, diethyl(3-chlorobenzyl)phosphonate, diethyl cyano-phosphonate, or diethyl phenylphosphonate.

#### Electrical Property Testing

The above prepared photoconductors of Comparative Examples 1(A) and 2(A), and Examples I and II were tested in a scanner set to obtain photoinduced discharge cycles, sequenced at one charge-erase cycle followed by one charge-expose-erase cycle, wherein the light intensity was incrementally increased with cycling to produce a series of photoinduced discharge characteristic (PIDC) curves from which the photosensitivity and surface potentials at various exposure intensities were measured. Additional electrical characteristics were obtained by a series of charge-erase cycles with incrementing surface potential to generate several voltages versus charge density curves. The scanner was equipped with a scorotron set to a constant voltage charging at various surface potentials. These two photoconductors were tested at surface potentials of 500 volts with the exposure light intensity incrementally increased by regulating a series of neutral density filters; the exposure light source was a 780 nanometer light emitting diode. The xerographic simulation was completed in an environmentally controlled light tight chamber at dry conditions (10 percent relative humidity and 22° C.).

The above prepared photoconductors exhibited substantially similar PIDCs. Thus, incorporation of the phosphonate into the hole blocking or undercoat layer did not adversely affect the electrical properties of the photoconductor.

#### Charge Deficient Spots (CDS) Measurement

Various known methods have been developed to assess and/or accommodate the occurrence of charge deficient spots. For example, U.S. Pat. Nos. 5,703,487 and 6,008,653, the disclosures of each patent being totally incorporated herein by reference, disclose processes for ascertaining the micro-defect levels of an electrophotographic imaging member or photoconductor. The method of U.S. Pat. No. 5,703,487, designated as field-induced dark decay (FIDD), involves measuring either the differential increase in charge over and above the capacitive value, or measuring reduction in voltage below the capacitive value of a known imaging member and of a virgin imaging member, and comparing differential increase in charge over and above the capacitive value or the reduction in voltage below the capacitive value of the known imaging member and of the virgin imaging member.

U.S. Pat. No. 6,008,653, recited above, and U.S. Pat. No. 6,150,824, the disclosures of each patent being totally incorporated herein by reference, disclose a method for detecting surface potential charge patterns in an electrophotographic imaging member with a floating probe scanner. Floating Probe Micro Defect Scanner (FPS) is a contactless process for detecting surface potential charge patterns in an electrophotographic imaging member. The scanner includes a capacitive probe having an outer shield electrode, which

maintains the probe adjacent to and spaced from the imaging surface to form a parallel plate capacitor with a gas between the probe and the imaging surface, a probe amplifier optically coupled to the probe, establishing relative movement between the probe and the imaging surface, and a floating fixture which maintains a substantially constant distance between the probe and the imaging surface. A constant voltage charge is applied to the imaging surface prior to relative movement of the probe and the imaging surface past each other, and the probe is synchronously biased to within about ±300 volts of the average surface potential of the imaging surface to prevent breakdown, measuring variations in surface potential with the probe, compensating the surface potential variations for variations in distance between the probe and the imaging surface, and comparing the compensated voltage values to a baseline voltage value to detect charge patterns in the electrophotographic imaging member. This process may be conducted with a contactless scanning system comprising a high resolution capacitive probe, a low spatial resolution electrostatic voltmeter coupled to a bias voltage amplifier, and an imaging member having an imaging surface capacitively coupled to and spaced from the probe and the voltmeter. The probe comprises an inner electrode surrounded by and insulated from a coaxial outer Faraday shield electrode, the inner electrode connected to an opto-coupled amplifier, and the Faraday shield connected to the bias voltage amplifier. A threshold of 20 volts is commonly chosen to count charge deficient spots. The above prepared photoconductors (Comparative Examples 1(A) and 2(A), Examples I and II) were measured for CDS counts using the above-described FPS technique, and the results follow in Table 1.

TABLE 1

|                                                                | Ground Plane | CDS (Counts/cm <sup>2</sup> ) |
|----------------------------------------------------------------|--------------|-------------------------------|
| Comparative Example 1 (A) With Aminosilane Hole Blocking Layer | Ti/Zr        | 18                            |
| Comparative Example 2 (A) With Aminosilane Hole Blocking Layer | Gold         | 132                           |
| Example I With Aminosilane/Phosphonate Hole Blocking Layer     | Gold         | 25                            |
| Example II With Aminosilane/Phosphonate Hole Blocking Layer    | Gold         | 19                            |

The aminosilane hole blocking layer was sufficient to block holes from the Ti/Zr ground plane, thus resulting in low CDS counts, specifically about 18 counts/cm<sup>2</sup> of Comparative Example 1(A). However, the same hole blocking layer was insufficient to block holes from a gold ground plane resulting in high CDS counts, specifically about 132 counts/cm<sup>2</sup> of Comparative Example 2(A).

With a gold ground plane, the above data with the phosphonate incorporated into the aminosilane hole blocking layer improved hole blocking. As a result, by incorporating the above phosphonates into the aminosilane hole blocking layer (Examples I and II), the CDS counts were reduced to about 25 and 19 counts/cm<sup>2</sup>, respectively, which were very comparable to that of the aminosilane hole blocking layer deposited on a Ti/Zr ground plane of Comparative Example 1(A).

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of

claims should not be implied or imported from the specification or any other claims as to any particular order, number, position, size, shape, angle, color, or material.

What is claimed is:

1. A photoconductor consisting essentially of a substrate; a ground plane layer; an undercoat layer thereover wherein the undercoat layer comprises an aminosilane and a phosphonate; a photogenerating layer; and at least one charge transport layer, and wherein said phosphonate is represented by



wherein R<sub>1</sub> is alkyl or aryl; and R<sub>2</sub> and R<sub>3</sub> are each independently at least one of hydrogen, alkyl, and aryl.

2. A photoconductor in accordance with claim 1 wherein said ground plane is gold.

3. A photoconductor in accordance with claim 1 wherein said ground plane is comprised of a gold containing material.

4. A photoconductor in accordance with claim 1 wherein said aminosilane is present in an amount of from about 50 to about 99.9 weight percent, said phosphonate is present in an amount of from about 0.1 to about 50 weight percent, and wherein the total of said components in said undercoat layer is about 100 percent.

5. A photoconductor in accordance with claim 1 wherein said aminosilane is present in an amount of from about 70 to about 99 weight percent; said phosphonate is present in an amount of from about 1 to about 30 weight percent; and wherein the total of said components in said undercoat layer is about 100 percent.

6. A photoconductor in accordance with claim 1 wherein said aminosilane is represented by a



wherein R<sub>1</sub> is an alkylene group containing from 1 to about 25 carbon atoms; R<sub>2</sub> and R<sub>3</sub> are independently selected from the group consisting of at least one of hydrogen, alkyl containing from 1 to about 5 carbon atoms, aryl containing from about 6 to about 36 carbon atoms, and a poly(alkylene amino) group; and R<sub>4</sub>, R<sub>5</sub>, and R<sub>6</sub> are independently selected from an alkyl group containing from 1 to about 6 carbon atoms.

7. A photoconductor in accordance with claim 1 wherein said aminosilane is at least one of 3-aminopropyl triethoxysilane, N,N-dimethyl-3-aminopropyl triethoxysilane, N-phenylaminopropyl trimethoxysilane, triethoxysilylpropylethylene diamine, trimethoxysilylpropylethylene diamine, trimethoxysilylpropylidene triamine, N-aminoethyl-3-aminopropyl trimethoxysilane, N-2-aminoethyl-3-aminopropyl trimethoxysilane, N-2-aminoethyl-3-aminopropyl tris(ethylethoxy)silane, p-aminophenyl trimethoxysilane, N,N'-dimethyl-3-aminopropyl triethoxysilane, 3-aminopropylmethyl diethoxysilane, 3-aminopropyl trimethoxysilane, N-methylaminopropyl triethoxysilane, methyl[2-(3-trimethoxysilylpropylamino)ethylamino]-3-propionate, (N,N'-dimethyl 3-amino)propyl triethoxysilane, N,N-dimethylaminophenyl triethoxysilane, trimethoxysilyl

propyldiethylene triamine, and mixtures thereof; and said at least one charge transport layer is 1, 2, 3, or 4 layers.

8. A photoconductor in accordance with claim 1 wherein R<sub>1</sub> is alkyl; and R<sub>2</sub> and R<sub>3</sub> are each independently at least one alkyl, and aryl.

9. A photoconductor in accordance with claim 1 wherein said phosphonate is at least one of N,N-bis-(2-hydroxylethyl) aminomethanephosphonic acid diethyl ester, (methylthiomethyl)phosphonic acid diethyl ester, 2-hydroxyethylphosphonic acid dimethyl ester, cyanomethylphosphonic acid diethyl ester, di-n-butyl N,N-diethylcarbamoylmethylphosphonate, dibutyl N,N-diethylcarbamoylphosphonate, diethyl(phthalimidomethyl)phosphonate, diethyl 1-pyrrolidinemethylphosphonate, diethyl 3,5-di-tert-butyl-4-hydroxybenzyl phosphonate, diphenyl (2,3-dihydro-2-thioxo-3-benzoxazolyl)phosphonate, monoethyl 3,5-di-tert-butyl-4-hydroxybenzylphosphonate, tetraethyl[4,4'-biphenylylenebis(methylene)]bisphosphonate,

4-methoxyphenylphosphonate, tetraethyl[anthracene-9,10-diylbis(methylene)]bisphosphonate, diethyl benzylphosphonate, bis(2,2,2-trifluoroethyl) (methoxycarbonylmethyl) phosphonate, diethyl phenacylphosphonate, diethyl (3-chlorobenzyl)phosphonate, diethyl cyanophosphonate, and diethyl phenylphosphonate.

10. A photoconductor in accordance with claim 1 wherein said undercoat layer further comprises an acid present in an amount of from about 50 to about 150 mole percent of said aminosilane.

11. A photoconductor in accordance with claim 1 wherein said undercoat layer is prepared by (a) hydrolyzing said aminosilane in water; (b) adding an acid thereto; and (c) adding said phosphonate, and wherein said acid is selected from the group consisting of acetic acid, citric acid, formic acid, hydrogen iodide, phosphoric acid, hydrofluorosilicic acid, and p-toluene sulfonic acid.

12. A photoconductor in accordance with claim 1 wherein said aminosilane is 3-aminopropyl triethoxysilane, and said phosphonate is N,N-bis-(2-hydroxylethyl)aminomethane phosphonic acid diethyl ester or diethyl(phthalimidomethyl) phosphonate, and the weight ratio thereof of said amino silane to said phosphate is from about 60/40 to about 95/5.

13. A photoconductor in accordance with claim 1 wherein the thickness of the undercoat layer is from about 0.01 micron to about 1 micron.

14. A photoconductor in accordance with claim 1 wherein the thickness of the undercoat layer is from about 0.04 micron to about 0.5 micron.

15. A photoconductor in accordance with claim 1 wherein said charge transport layer is comprised of at least one of



27

-continued



wherein X, Y, and Z are independently selected from the group consisting of alkyl, alkoxy, aryl, halogen, and mixtures thereof.

**16.** A photoconductor in accordance with claim 1 wherein said charge transport layer is comprised of a component selected from the group consisting of N,N'-bis(methylphenyl)-1,1-biphenyl-4,4'-diamine, N,N'-bis(4-butylphenyl)-N, N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-[p-terphenyl]-4,4'-diamine, N,N'-bis(4-butylphenyl)-N, N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, and N,N'-diphenyl-N,N'-bis(3-chlorophenyl)-[p-terphenyl]-4,4'-diamine; and said at least one charge transport layer is 1, 2, or 3 layers.

**17.** A photoconductor in accordance with claim 1 wherein said photogenerating layer is comprised of at least one photogenerating pigment.

**18.** A photoconductor in accordance with claim 17 wherein said photogenerating pigment is comprised of at least one of a titanyl phthalocyanine, a hydroxygallium phthalocyanine, a halogallium phthalocyanine, a bisperylene, and mixtures thereof.

**19.** A photoconductor in accordance with claim 1 wherein said at least one charge transport layer is comprised of a charge transport component and a resin binder, and wherein said photogenerating layer is comprised of at least one photogenerating pigment and a resin binder; and wherein said photogenerating layer is situated between said substrate and said charge transport layer; and wherein said aminosilane is represented by



wherein R<sub>1</sub> is an alkylene group containing from 1 to about 25 carbon atoms; R<sub>2</sub> and R<sub>3</sub> are independently selected from the group consisting of at least one of hydrogen, alkyl containing from 1 to about 5 carbon atoms, aryl containing from about 6 to about 36 carbon atoms, and a poly(alkylene amino) group; and R<sub>4</sub>, R<sub>5</sub>, and R<sub>6</sub> are independently selected from an alkyl group containing from 1 to about 6 carbon atoms; and said phosphonate is at least one of N,N-bis-(2-hydroxyethyl)aminomethanephosphonic acid diethyl ester, (methylthiomethyl)phosphonic acid diethyl ester, 2-hydroxyethylphosphonic acid dimethyl ester, cyanomethylphosphonic acid diethyl ester, di-n-butyl N,N-diethylcarbamoylmethylphosphonate, dibutyl N,N-diethylcarbamoylphosphonate, diethyl(phthalimidomethyl)phosphonate, diethyl 1-pyrrolidinemethylphosphonate, diethyl 3,5-di-tert-butyl-4-hydroxybenzyl phosphonate, diphenyl (2,3-dihydro-2-thioxo-3-benzoxazolyl)phosphonate, monoethyl 3,5-di-tert-butyl-4-hydroxybenzylphosphonate, tetraethyl[4,4'-biphenylenebis(methylene)]bisphosphonate, diethyl 4-methoxyphenylphosphonate, tetraethyl [anthracene-9,10-diylbis(methylene)]bisphosphonate, diethyl benzylphosphonate, bis(2,2,2-trifluoroethyl) (methoxycarbonylmethyl) phosphonate, diethyl phenacylphosphonate, diethyl (3-chlorobenzyl)phosphonate, diethyl cyanophosphonate, and diethyl phenylphosphonate.

**28**  
 acid dimethyl ester, cyanomethylphosphonic acid diethyl ester, di-n-butyl N,N-diethylcarbamoylmethylphosphonate, dibutyl N,N-diethylcarbamoylphosphonate, diethyl(phthalimidomethyl)phosphonate, diethyl 1-pyrrolidinemethylphosphonate, diethyl 3,5-di-tert-butyl-4-hydroxybenzyl phosphonate, diphenyl (2,3-dihydro-2-thioxo-3-benzoxazolyl)phosphonate, monoethyl 3,5-di-tert-butyl-4-hydroxybenzylphosphonate, tetraethyl[4,4'-biphenylenebis(methylene)]bisphosphonate, diethyl 4-methoxyphenylphosphonate, tetraethyl [anthracene-9,10-diylbis(methylene)]bisphosphonate, diethyl benzylphosphonate, bis(2,2,2-trifluoroethyl) (methoxycarbonylmethyl) phosphonate, diethyl phenacylphosphonate, diethyl (3-chlorobenzyl)phosphonate, diethyl cyanophosphonate, and diethyl phenylphosphonate.

**20.** A photoconductor consisting essentially of a substrate; a ground plane layer; an undercoat layer thereover comprised of a mixture of an aminosilane and a phosphonate; a photogenerating layer; and a charge transport layer, and wherein said phosphonate is N,N-bis-(2-hydroxyethyl)aminomethanephosphonic acid diethyl ester, (methylthiomethyl)phosphonic acid diethyl ester, 2-hydroxyethylphosphonic acid dimethyl ester, cyanomethylphosphonic acid diethyl ester, di-n-butyl N,N-diethylcarbamoylmethylphosphonate, dibutyl N,N-diethylcarbamoylphosphonate, diethyl(phthalimidomethyl)phosphonate, diethyl 1-pyrrolidinemethylphosphonate, diethyl 3,5-di-tert-butyl-4-hydroxybenzylphosphonate, diphenyl (2,3-dihydro-2-thioxo-3-benzoxazolyl)phosphonate, monoethyl 3,5-di-tert-butyl-4-hydroxybenzyl phosphonate, tetraethyl[4,4'-biphenylenebis(methylene)]bisphosphonate, diethyl 4-methoxyphenylphosphonate, tetraethyl [anthracene-9,10-diylbis(methylene)]bisphosphonate, diethyl benzylphosphonate, bis(2,2,2-trifluoroethyl) (methoxycarbonylmethyl) phosphonate, diethyl phenacylphosphonate, diethyl (3-chlorobenzyl)phosphonate, diethyl cyanophosphonate, or diethyl phenylphosphonate.

**21.** A photoconductor in accordance with claim 20 wherein said phosphonate is N,N-bis-(2-hydroxyethyl)aminomethanephosphonic acid diethyl ester, (methylthiomethyl)phosphonic acid diethyl ester, or diethyl(phthalimidomethyl)phosphonate, and said aminosilane is an aminoalkyl alkoxy silane.

**22.** A photoconductor in accordance with claim 20 wherein said phosphonate is N,N-bis-(2-hydroxyethyl)aminomethanephosphonic acid diethyl ester or diethyl(phthalimidomethyl)phosphonate, and said aminosilane is 3-amino-propyl triethoxysilane.

**23.** A photoconductor consisting essentially of and in sequence a supporting substrate; a gold containing ground plane layer; a hole blocking layer comprised of an aminosilane and a phosphonate mixture; a photogenerating layer; and a charge transport layer containing continuously throughout said layer from about 10 to about 75 weight percent of a charge transport compound, and wherein said phosphonate is selected from the group consisting of N,N-bis-(2-hydroxyethyl)aminomethanephosphonic acid diethyl ester, (methylthiomethyl)phosphonic acid diethyl ester, 2-hydroxyethylphosphonic acid dimethyl ester, cyanomethylphosphonic acid diethyl ester, di-n-butyl N,N-diethylcarbamoylmethylphosphonate, dibutyl N,N-diethylcarbamoylphosphonate, diethyl(phthalimidomethyl)phosphonate, diethyl 1-pyrrolidinemethylphosphonate, diethyl 3,5-di-tert-butyl-4-hydroxybenzylphosphonate, diphenyl (2,3-dihydro-2-thioxo-3-benzoxazolyl)phosphonate, monoethyl 3,5-di-tert-butyl-4-hydroxybenzyl phosphonate, tetraethyl[4,4'-biphenylenebis(methylene)]bisphosphonate, diethyl 4-methoxyphenylphosphonate, tetraethyl [anthracene-9,10-diylbis(methylene)]bisphosphonate, diethyl benzylphosphonate, bis(2,2,2-trifluoroethyl) (methoxycarbonylmethyl)

29

phosphonate, diethyl phenacylphosphonate, diethyl (3-chlorobenzyl)phosphonate, diethyl cyanophosphonate, and diethyl phenylphosphonate.

24. A photoconductor in accordance with claim 23 wherein said aminosilane is at least one of 3-aminopropyl triethoxysilane, N,N-dimethyl-3-aminopropyl triethoxysilane, N-phenylaminopropyl trimethoxysilane, triethoxysilylpropylethylene diamine, trimethoxysilylpropylethylene diamine, trimethoxysilylpropyl diethylene triamine, N-aminoethyl-3-aminopropyl trimethoxysilane, N-2-aminoethyl-3-aminopropyl trimethoxysilane, N-2-aminoethyl-3-aminopropyl triis(ethylethoxy)silane, p-aminophenyl trimethoxysilane, N,N'-dimethyl-3-aminopropyl triethoxysilane, 3-aminopropylmethyl diethoxysilane, 3-aminopropyl trimethoxysilane, N-methylaminopropyl triethoxysilane, methyl[2-(3-trimethoxysilylpropylamino)ethylamino]-3-propionate, (N,N'-dimethyl 3-amino)propyl triethoxysilane, N,N-dimethylaminophenyl triethoxysilane, trimethoxysilylpropyl diethylene triamine, and mixtures thereof, and wherein said phosphonate is selected from the group consisting of N,N-bis-(2-hydroxylethyl)aminomethane phosphonic acid diethyl ester and diethyl (phthalimidomethyl)phosphonate.

25. A photoconductor in accordance with claim 1 wherein said undercoat layer further contains a resin binder selected from the group consisting of polyacetal resins, polyvinyl butyral resins, aminoplast resins, melamine resins, and mixtures thereof. 25

**26.** A photoconductor in accordance with claim 1 wherein said aminosilane is an aminoalkyl trialkoxy silane.

27. A photoconductor in accordance with claim 1 wherein said ground plane is gold, said phosphonate is N,N-bis(2-hydroxyethyl)aminomethane phosphonic acid diethyl ester, said charge transport layer is comprised of an aryl amine and a polymeric binder; and said silane is an aminoalkyltrialkoxysilane.

28. A photoconductor in accordance with claim 1 wherein said ground plane is gold, said phosphonate is diethyl(phthalimidomethyl)phosphonate, said charge transport layer is comprised of an aryl amine and a polymeric binder; and said silane is an aminoalkyltrialkoxysilane.

29. A photoconductor in accordance with claim 20 wherein said aminosilane is represented by



wherein  $R_1$  is an alkylene;  $R_2$  and  $R_3$  are alkyl, hydrogen, aryl, or a poly(alkyleneamino) group; and each  $R_4$ ,  $R_6$ , and  $R_7$  is alkyl.

30. A photoconductor in accordance with claim 20 wherein 55  
said phosphonate is represented by at least one of



30

-continued



**31**

-continued

**32**

-continued



\* \* \* \* \*